

## UNITED STATES PATENT OFFICE

2,543,841

METAL ALLOY ESPECIALLY ADAPTED FOR  
USE AT HIGH TEMPERATURESFrancis B. Foley, Philadelphia, Pa., assignor to  
The Midvale Company, Philadelphia, Pa., a corporation of DelawareNo Drawing. Application June 26, 1948,  
Serial No. 35,533

5 Claims. (Cl. 75—134)

1

My invention comprises a metal alloy for use at elevated temperatures such as are experienced in gas turbines and which is believed to excel other alloys heretofore made in the following respects:

1. It has a higher combination of creep strength, fracture time for a given load and temperature, fatigue strength and resistance to scaling at high temperatures.

2. Resistance to grain growth.

3. Ease of hot working.

Alloys intended and adapted for the above special use having compositions containing the same constituents as my improved alloy are known in the art. My improved alloy, however, differs from these known alloys in several essential respects. All such alloys contain a substantial percentage of molybdenum, which, for reasons hereinafter explained, must not be present in my al-

loyage of iron will hardly exceed ten per cent. With minimum permissible proportions of the other constituents the percentage of iron will not exceed about 25 per cent. In fact, nickel, chromium, and iron are largely interchangeable if the percentages of nickel and chromium are maintained within the above limits. The presence of some iron is therefore desirable. It is also desirable from the standpoint of economy of manufacture and could hardly be practically excluded when, as is usual, certain alloying metals are, in commercial form, alloyed with iron.

Manganese and silicon are not essential constituents, but their exclusion is difficult and their presence in small proportions does not impair the qualities characteristic of my improved alloy.

I have found it distinctly advantageous to keep the proportions of the several ingredients within the following ranges:

| C       | Mn     | Si     | Ni    | Cr    | Co    | W     | Cb    | N       | Fe   |
|---------|--------|--------|-------|-------|-------|-------|-------|---------|------|
| .10-.30 | .5-1.0 | .5-1.0 | 31-35 | 18-22 | 27-32 | 5.5-8 | 2.5-4 | .10-.20 | bal. |

loy in any substantial proportion and which is, decidedly preferably, excluded altogether. If present at all its permissible proportion should

An alloy that is particularly acceptable for commercial use has the following approximate composition:

| C   | Mn  | Si  | Ni   | Cr   | Co    | W    | Cb   | N   | Fe   |
|-----|-----|-----|------|------|-------|------|------|-----|------|
| .20 | .72 | .78 | 32.5 | 20.0 | 29.25 | 6.30 | 3.50 | .15 | bal. |

be substantially less than one per cent. My improved alloy, as in other alloys intended for similar uses, contains tungsten, but in a higher than usual percentage, the tungsten and nitrogen combining to control grain growth. It also is distinguished from such other alloys by its high nickel content.

The constituents of my improved alloy, with the maximum percentage ranges of the constituents, is as follows:

This composition, with little deviation from the proportions given, is distinctly preferred.

35 The main objection to carbon approximating 1.5% is that high carbon requires great care in heating and working. Even in forging one could, with difficulty, forge up to 1% of carbon and possibly up to near 1.5%. To avoid hot working difficulties and consequent uncertainty of results the percentage of carbon should not exceed .50 per cent and it is desirably considerably lower, while

| C          | Mn        | Si        | Ni    | Cr    | Co    | W   | Cb  | N       | Fe   |
|------------|-----------|-----------|-------|-------|-------|-----|-----|---------|------|
| up to 1.50 | up to 1.5 | up to 1.5 | 30/40 | 18/24 | 17/35 | 4/8 | 2/6 | .10/.20 | bal. |

Iron is not essential. When the other constituents are present in preferred proportions the per-

centage in forgings the carbon percentage should not exceed .30 per cent. It is also highly desirable to

maintain a proper carbon-cobalt balance, as hereinafter explained, which, in the case of a desirably high cobalt percentage, requires a comparatively low carbon content.

Vanadium in my composition is an equivalent of tungsten and may replace it in whole or in part, but in the ratio of one part of vanadium to two parts of tungsten.

While in most alloys tungsten and molybdenum function as equivalents they are not such in my composition. Molybdenum cannot be substituted even in part for tungsten and in my alloy is merely one of a number of elements which might be added in unsubstantial proportions without appreciable benefit and without pronounced harm.

There are two principal reasons for excluding molybdenum, or, to express it otherwise, molybdenum has two undesirable effects when a constituent of metallic alloys subjected to elevated temperatures. One of the changes in structure at elevated temperatures which gives rise to embrittlement in alloys of the type covered by this invention is the formation of a non-magnetic very hard phase identical in crystalline structure with the brittle sigma phase found in iron-chromium and iron-nickel-chromium alloys. Molybdenum is twice as active as tungsten in developing this brittle phase and I find tungsten in this alloy to be as effective as molybdenum in conferring resistance to deformation in the alloy.

The other undesirable effect of molybdenum is in its lowering of the resistance of the metal to oxidation at high temperatures. Under certain conditions of exposure molybdenum can lead to the complete destruction of the metal by its conversion to oxide in an extremely short period of time. Such rapid oxidation has been called "catastrophic oxidation."

The use of tungsten as a strengthener avoids these undesirable effects and promotes forgeability.

The presence of nitrogen in amounts of .10 to .20% restrains grain growth.

It is generally recognized that coarse grain size promotes resistance to deformation at high temperatures and that a fine grain structure is relatively weak at high temperatures. I find that this fine grain characteristic of metals can be taken advantage of in my alloy to render it more readily responsive to deformation in hot working and that the coarse grain advantage in strengthening can be provided by means of a heat treatment involving exposure of the alloy to a temperature high enough to produce a desirable larger grain size. This property of the alloy of lending itself readily to hot working makes hot forging, in either open or closed dies, and rolling, both practical and economical. Turbine blading sections have been produced by drop forging, and the alloy under such conditions of working has been found to be extremely ductile and to display a degree of forgeability greater than any of the currently used alloys designed for gas turbine blading. This was evident from the ability of the metal to withstand a greater degree of deformation without splitting or fracturing than in turbine bucket metal heretofore used.

The most serious weakening of the crystalline structure at high temperatures results from active grain growth. Therefore an alloy which resists grain growth will have less active grain boundaries and thus resist deformation more effectively than one which undergoes relatively rapid grain-growth. My composition in the wrought conditions attains an A. S. T. M. grain

size of only 4 or 5 after exposure at 2375° F., which is the highest temperature to which it would be exposed for coarsening; higher temperature involving a risk of reaching the solidus of the alloy and thus producing physical damage and a weakening of the structure.

When melted to the preferred analysis this alloy will hold a load of 17,000 p. s. i. in tension at 1500° F. for 1000 hours and in fatigue at this temperature it withstands 100 million reversals of a stress of 42,000 p. s. i. before failure occurs.

I find that the carbon content of the alloy has a great influence on the resistance of the metal to failure under load at elevated temperatures.

Over the limits between 0.15% and 0.30%, carbon is more effective in strengthening the alloy than is cobalt within the range 17.0 to 30.0%. However, this advantage of carbon is limited by the increased difficulty with which the alloy is hot worked as the carbon increases. Thus, for maintaining strength at high temperature, carbon may be increased as the cobalt is decreased, but strength thus obtained is at the sacrifice of hot working properties and such high carbon alloys are best suited for use as castings, whereas the high cobalt-low carbon combination is better suited to a wrought product. The effect of carbon and cobalt is shown in the following table:

|   | C   | Ni   | Cr   | Co   | W    | Cb   | N   | Stress in p. s. i., producing failure in 1000 hours |
|---|-----|------|------|------|------|------|-----|-----------------------------------------------------|
| A | .22 | 33.0 | 20.8 | 29.5 | 7.20 | 2.92 | .13 | 16,900                                              |
| B | .29 | 31.2 | 19.8 | 17.6 | 6.75 | 3.15 | .12 | 14,600                                              |
| C | .17 | 33.3 | 18.4 | 29.3 | 7.44 | 3.15 | .18 | 14,200                                              |

Alloy B represents a relatively high carbon, low cobalt combination and has about the same strength as alloy C with lower carbon and higher cobalt. Alloy A, in which the carbon and cobalt are balanced to produce good hot working properties, gives the highest values. Alloy A, it will be observed, is almost identical in composition, in its high nickel and high tungsten content, as well as in its carbon-cobalt balance, with the preferred specific composition hereinbefore given.

What I claim and desire to protect by Letters Patent is:

1. A metal alloy especially useful as a composition for structures, such as gas turbines, normally subjected to high temperature consisting essentially of carbon not exceeding 1.50 per cent., small percentages of manganese and silicon, nickel 30 to 40 per cent., chromium 18 to 24 per cent., cobalt 17 to 35 per cent., tungsten 4 to 8 per cent., molybdenum 0 to substantially less than one per cent., columbium over 2 and not over 6 per cent., nitrogen .10 to .20 per cent., the remainder substantially all iron, the percentage of the ingredients other than iron being such, within the specified limits, that the proportion of iron does not exceed 25%.

2. A metal alloy especially useful as a composition for structures, such as gas turbines, normally subjected to high temperatures consisting essentially of carbon .10 to .30 per cent., small percentages of manganese and silicon, nickel 31 to 35 per cent., chromium 18 to 22 per cent., cobalt over 27 and not over 32 per cent., tungsten 5.5 to 8 per cent., molybdenum 0 to substantially less than one per cent., columbium 2.5 to 4 per cent., nitrogen .10 to .20 per cent., the remainder substantially all iron, the percentage of the ingredients other than iron being such, within the

specified ranges, that the proportion of iron does not exceed 14%.

3. A metal alloy of the composition specified in claim 2 in which the percentage of carbon is between 0.19 and 0.23 per cent. and the percentage of cobalt is between 120 and 160 times the percentage of carbon.

4. A metal alloy especially useful as a composition for structures, such as gas turbines, normally subjected to high temperatures consisting essentially of the following constituents in approximately the following proportions: carbon .19-.23 per cent., manganese and silicon each between .5 to 1.0 per cent., nickel 31-34 per cent., chromium 19.5-21.5 per cent., cobalt 28.5-31.5 per cent., tungsten 6.0-7.5 per cent., molybdenum 0 to substantially less than one per cent., columbium 2.75-3.9 per cent., nitrogen about .15 per cent., iron 5 to 10%, and no substantial proportion of any other constituent.

5. A metal alloy especially useful as a composition for structures, such as gas turbines, normally subjected to high temperatures consisting

essentially of carbon 0.27-0.30 per cent., small percentages of manganese and silicon, nickel 31 to 35 per cent., chromium 18 to 22 per cent., cobalt 17 to 20 per cent., tungsten 5.5 to 8 per cent., columbium 2.5 to 4 per cent., nitrogen 0.10 to 0.20 per cent., the remainder substantially all iron.

FRANCIS B. FOLEY.

#### REFERENCES CITED

The following references are of record in the file of this patent:

#### UNITED STATES PATENTS

| Number       | Name                | Date          |
|--------------|---------------------|---------------|
| 15 2,246,078 | Rohn et al. -----   | June 17, 1941 |
| 2,432,618    | Franks et al. ----- | Dec. 16, 1947 |

#### OTHER REFERENCES

- Progress Report on "Heat Resisting Metals for  
20 Gas Turbine Parts" (N-102); P. B. No. 39, 579;  
Sept. 21, 1943; stamped: "declassified to open Feb.  
18, 1946," page 6.